

## 1

3,303,236

## UNSATURATED HYDROCARBONS BY OXIDATIVE DEHYDROGENATION OVER CATALYSTS COMPRISING NICKEL AND IRON

Louis J. Croce, East Brunswick, and Laimonis Bajars, Princeton, N.J., assignors to Petro-Tex Chemical Corporation, Houston, Tex., a corporation of Delaware  
No Drawing. Filed Jan. 2, 1964, Ser. No. 335,364  
17 Claims. (Cl. 260—680)

This invention relates to a process for dehydrogenating organic compounds and relates more particularly to the dehydrogenation of hydrocarbons at elevated temperatures in the presence of oxygen and a particular catalyst.

We have now discovered that greatly improved yields and high selectivities of unsaturated hydrocarbons are obtained by dehydrogenating under certain specified conditions hydrocarbons in the vapor phase at elevated temperatures in the presence of oxygen and a catalyst containing nickel ferrite.

Nickel ferrite is a known commercial product which has uses such as in the formulation of coatings suitable for high temperature applications. One method for the production of nickel ferrite is by the addition of nickelous oxide to an aqueous slurry of yellow iron oxide hydrate with the reaction mixture containing a small amount of the hydrate of potassium chloride as a catalyst. This reaction composition is uniformly mixed and then heated at a relatively low temperature above 100° C. for a period of several hours. The composition is then reacted for about 30 minutes at a temperature of 900° C. The reaction product is then ground and pelleted into catalyst particles.

Hydrocarbons to be dehydrogenated according to the process of this invention are hydrocarbons of 4 to 7 carbon atoms and preferably are aliphatic hydrocarbons selected from the group consisting of saturated hydrocarbons, monoolefins, diolefins and mixtures thereof of 4 to 5 or 6 carbon atoms having a straight chain of at least four carbon atoms and cycloaliphatics. Examples of preferred feed materials are butene-1, cis-butene-2, trans-butene-2, 2-methylbutene-1, 2-methylbutene-2, 2-methylbutene-3, n-butane, butadiene-1,3, methyl butane, 2-methylpentene-1, cyclohexene, 2-methylpentene-2 and mixtures thereof. For example, n-butane may be converted to a mixture of butene-1 and butene-2 or may be converted to a mixture of butene-1, butene-2 and/or butadiene-1,3. A mixture of n-butane and butene-2 may be converted to butadiene-1,3 or to a mixture of butadiene-1,3 together with some butene-2 and butene-1. Vinyl acetylene may be present at a product, particularly when butadiene-1,3 is used as a feedstock. Thus, the process of this invention is useful in converting hydrocarbons to less saturated hydrocarbons of the same number of carbon atoms. The major proportion of the hydrocarbon converted will be to less saturated hydrocarbons of the same number of carbon atoms. Particularly the preferred products are butadiene-1,3 and isoprene. Useful feeds may be mixed hydrocarbon streams such as refinery streams, or the olefin containing hydrocarbon mixture obtained as the product from the dehydrogenation of hydrocarbons. In the production of gasoline from higher hydrocarbons by either thermal or catalytic cracking a hydrocarbon stream containing predominantly hydrocarbons of 4 carbon atoms may be produced and may comprise a mixture of butenes

## 2

together with butadiene, butane, isobutane, isobutylene and other ingredients in minor amounts. These and other refinery by-products which contain normal, ethylenically unsaturated hydrocarbons are useful as starting materials. Although various mixtures of hydrocarbons are useful, the preferred hydrocarbon feed contains at least 50 weight percent of a hydrocarbon selected from the group consisting of butene-1, butene-2, n-butane, butadiene-1,3, 2-methylbutene-1, 2-methylbutene-2, 2-methylbutene-3 and mixtures thereof, and more preferably contains at least 70 weight percent of one or more of these hydrocarbons (with both of these percentages being based on the total weight of the organic composition of the feed to the reactor). Any remainder may be, for example, essentially aliphatic hydrocarbons. This invention is particularly useful to provide a process whereby the major product of the hydrocarbon converted is a dehydrogenated hydrocarbon product having the same number of carbon atoms as the hydrocarbon fed.

Oxygen will be present in the reaction zone in an amount within the range of 0.2 to 2.5 mols of oxygen per mol of hydrocarbon to be dehydrogenated. Generally, better results may be obtained if the oxygen concentration is maintained between about 0.25 and about 1.6 mols of oxygen per mol of hydrocarbon to be dehydrogenated, such as between 0.35 and 1.2 mols of oxygen. The oxygen may be fed to the reactor as pure oxygen, as air, as oxygen-enriched air, oxygen mixed with diluents and so forth. Based on the total gaseous mixture entering the reactor, the oxygen ordinarily will be present in an amount from about 0.5 to 25 volume percent of the total gaseous mixture, and more usually will be present in an amount from about 1 to 15 volume percent of the total. The total amount of oxygen utilized may be introduced into the gaseous mixture entering the catalytic zone or sometimes it has been found desirable to add the oxygen in increments, such as to different sections of the reactor. The above described proportions of oxygen employed are based on the total amount of oxygen used. The oxygen may be added directly to the reactor or it may be premixed, for example, with a diluent or steam.

The temperature for the dehydrogenation reaction will be greater than 250° C., such as greater than about 300° C. or 375° C., and the maximum temperature in the reactor may be about 650° C. or 750° C. or perhaps higher under certain circumstances. However, excellent results are obtained within the range of or about 300° C. to 575° C. such as from or about 325° C. to or about 525° C. The temperatures are measured at the maximum temperature in the reactor. An advantage of this invention is that lower temperatures of dehydrogenation may be utilized than are possible in conventional dehydrogenation processes. Another advantage is that large quantities of heat do not have to be added to the reaction as was previously required.

The dehydrogenation reaction may be carried out at atmospheric pressure, superatmospheric pressure or at subatmospheric pressure. The total pressure of the system will normally be about or in excess of atmospheric pressure, although sub-atmospheric pressure may also desirably be used. Generally, the total pressure will be between about 4 p.s.i.a. and about 100 or 125 p.s.i.a. Preferably the total pressure will be less than about 75 p.s.i.a. and excellent results are obtained at about atmospheric pressure.

The initial partial pressure of the hydrocarbon to be dehydrogenated will be equivalent to less than one-half atmosphere at a total pressure of one atmosphere. Generally the combined partial pressure of the hydrocarbon to be dehydrogenated together with the oxygen will also be equivalent to less than one-half atmosphere at a total pressure of one atmosphere. Preferably, the initial partial pressure of the hydrocarbon to be dehydrogenated will be equivalent to no greater than one-third atmosphere or no greater than one-fifth atmosphere at a total pressure of one atmosphere. Also, preferably, the initial partial pressure of the combined hydrocarbon to be dehydrogenated plus the oxygen will be equivalent to no greater than one-third or no greater than one-fifth atmosphere at a total pressure of one atmosphere. Reference to the initial partial pressure of the hydrocarbon to be dehydrogenated means the partial pressure of the hydrocarbon as it first contacts the catalytic particles. An equivalent partial pressure at a total pressure of one atmosphere means that one atmosphere total pressure is a reference point and does not imply that the total pressure of the reaction must be operated at atmospheric pressure. For example, in a mixture of one mol of butene, three mols of steam, and one mol of oxygen under a total pressure of one atmosphere, the butene would have an absolute pressure of one-fifth of the total pressure, or roughly six inches of mercury absolute pressure. Equivalent to this six inches of mercury butene absolute pressure at atmospheric pressure would be butene mixed with oxygen under a vacuum such that the partial pressure of the butene is 6 inches of mercury absolute. The combination of a diluent such as nitrogen, together with the use of a vacuum may be utilized to achieve the desired partial pressure of the hydrocarbon. For the purpose of this invention, also equivalent to the six inches of mercury butene absolute pressure at atmospheric pressure would be the same mixture of one mol of butene, three mols of steam and one mol of oxygen under a total pressure greater than atmospheric, for example, a total pressure of 20 p.s.i.a. Thus, when the total pressure in the reaction zone is greater than one atmosphere, the absolute values for the pressure of the hydrocarbon to be dehydrogenated will be increased in direct proportion to the increase in total pressure above one atmosphere.

The partial pressures described above may be maintained by the use of diluents such as nitrogen, helium or other gases. Conveniently, the oxygen may be added as air with the nitrogen acting as a diluent for the system. Mixtures of diluents may be employed. Volatile compounds which are not dehydrogenated or which are dehydrogenated only to a limited extent may be present as diluents.

Preferably the reaction mixture contains a quantity of steam, with the range generally being between about 2 and 40 mols of steam per mol of hydrocarbon to be dehydrogenated. Preferably steam will be present in an amount from about 3 to 35 mols per mol of hydrocarbon to be dehydrogenated and excellent results have been obtained within the range of about 5 to about 30 mols of steam per mol of hydrocarbon to be dehydrogenated. The functions of the steam are several-fold, and the steam does not merely act as a diluent. Diluents generally may be used in the same quantities as specified for the steam. Excellent results are obtained when the gaseous composition fed to the reactor consists essentially of hydrocarbons, inert diluents and oxygen as the sole oxidizing agent.

The gaseous reactants may be conducted through the reaction chamber at a fairly wide range of flow rates. The optimum flow rate will be dependent upon such variables as the temperature of reaction, pressure, particle size, and whether a fluid bed or fixed bed reactor is utilized. Desirable flow rates may be established by one skilled in the art. Generally, the flow rates will be within the range of about 0.10 to 25 liquid volumes of the hydrocarbon to be dehydrogenated per volume of reactor containing

catalyst per hour (referred to as LHSV), wherein the volumes of hydrocarbon are calculated at standard conditions of 25° C. and 760 mm. of mercury. Usually, the LHSV will be between 0.15 and about 5 or 10. For calculation, the volume of reactor containing catalyst is that volume of reactor space excluding the volume displaced by the catalyst. For example, if a reactor has a particular volume of cubic feet of void space, when that void space is filled with catalyst particles, the original void space is the volume of reactor containing catalyst for the purpose of calculating the flow rate. The gaseous hourly space velocity (GHSV) is the volume of the hydrocarbon to be dehydrogenated in the form of vapor calculated under standard conditions of 25° C. and 760 mm. of mercury per volume of reactor space containing catalyst per hour. Generally, the GHSV will be between about 25 and 6400, and excellent results have been between about 38 and 3800. Suitable contact times are, for example, from about 0.001 or higher to about 5 or 10 seconds, with particularly good results being obtained between 0.01 and 3 seconds. The contact time is the calculated dwell time of the reaction mixture in the reaction zone, assuming the mols of product mixture are equivalent to the mols of feed mixture. For the purpose of calculation of residence times, the reaction zone is the portion of the reactor containing catalyst.

The catalytic surface described is the surface which is exposed in the dehydrogenation zone to the reactor, that is, if a catalyst carrier is used, the composition described as a catalyst refers to the composition of the surface and not to the total composition of the surface coating plus carrier. Catalyst binding agents or fillers may be used, but these will not ordinarily exceed about 50 percent or 60 percent by weight of the catalytic surface. These binding agents and fillers will preferably be essentially inert. The quantity of catalyst utilized will be dependent upon such variables as the temperature of reaction, the concentration of oxygen, the age of the catalyst, and the flow rates of the reactants. The catalyst will by definition be present in a catalytic amount and generally the nickel ferrite together with any nickel and iron atoms not combined as nickel ferrite will be the main active constituents. The amount of catalyst will ordinarily be present in an amount greater than 10 square feet of catalyst surface per cubic foot of reaction zone containing catalyst. Of course, the amount of catalyst may be much greater, particularly when irregular surface catalysts are used. When the catalyst is in the form of particles, either supported or unsupported, the amount of catalyst surface may be expressed in terms of the surface area per unit weight of any particular volume of catalyst particles. The ratio of catalytic surface to weight will be dependent upon various factors, including the particle size, particle size distribution, apparent bulk density of the particles, amount of active catalyst coated on the carrier, density of the carrier, and so forth. Typical values for the surface to weight ratio are such as about one-half to 200 square meters per gram, although higher and lower values may be used.

The dehydrogenation reactor may be of the fixed bed or fluid bed type. Conventional reactors for the production of unsaturated hydrocarbons are satisfactory. Excellent results have been obtained by packing the reactor with catalyst particles as the method of introducing the catalytic surface. The catalytic surface may be introduced as such or it may be deposited on a carrier by methods known in the art such as by preparing an aqueous solution or dispersion of a catalytic material and mixing the carrier with the solution or dispersion until the active ingredients are coated on the carrier. If a carrier is utilized, very useful carriers are silicon carbide, pumice and the like. When carriers are used, the amount of catalyst on the carrier will generally be between about 5 to 75 weight percent of the total weight of the active catalytic material plus carrier. Another method for in-

roducing the required surface is to utilize as a reactor a small diameter tube wherein the tube wall is catalytic or is coated with catalytic material. Other methods may be utilized to introduce the catalytic surface such as by the use of rods, wires, mesh, or shreds and the like of catalytic material.

According to this invention, the catalyst is autoregenerative and the process is continuous. Moreover, small amounts of tars and polymers are formed as compared to some prior art processes.

In the following examples will be found specific embodiments of the invention and details employed in the practice of the invention. Percent conversion refers to the mols of hydrocarbon consumed per 100 mols of hydrocarbon fed to the reactor, percent selectively refers to the mols of product formed per 100 mols of hydrocarbon consumed, and percent yield refers to the mols of product formed per mol of hydrocarbon fed.

#### EXAMPLE 1

A nickel ferrite catalyst was prepared from 37.4 grams of nickelous oxide, 79.9 grams ferric oxide and 74.6 grams of potassium chloride. The dry ingredients were mixed thoroughly and then reacted at 900° C. for a period of 1½ hours. After cooling to room temperature, hot distilled water was used to extract the potassium chloride from the reacted mixture. A highly magnetic dark brown solid was obtained after the reaction mixture was dried in an oven at 110° C. The product was found to be nickel ferrite by X-ray diffraction analysis.

The nickel ferrite was coated on 4 to 5 mesh alumina supports (Carborundum Company type AMC). Butene-2 was dehydrogenated at atmospheric pressure in a Vycor<sup>1</sup> glass reactor (36" x 1" O.D.) having a 35 cc. catalyst bed. The remainder of the reactor was filled with ¼" x ¼" Vycor Raschig rings. Butene-2, oxygen, and steam were introduced into an adapter located on top of the glass reactor, and the effluent gases were passed through a cold water condenser to remove most of the steam. Samples of the effluent gases were withdrawn with a syringe at the exit from the condenser. They were analyzed in a vapor chromatograph. The temperature inside the reactor was measured by a type J iron-constantan thermocouple enclosed in a 7 mm. O.D. Vycor tubing thermocouple well. The oxygen was fed as C.P. oxygen, 99.5 mol percent minimum oxygen.

The butene-2, oxygen and steam was fed to the reactor in an amount of 0.6 mol of oxygen per mol of butene-2 and 30 mols of steam per mol of butene-2. The liquid hourly space velocity was 1.0 (with the calculation being based on the volume of the reactor containing catalyst, that is, the 35 cc. catalyst section). At a maximum temperature in the reactor of 470° C., the yield of butadiene-1,3 was 64 mol percent per pass.

An X-ray diffraction pattern was obtained on the catalyst of Example 1. The powder pattern was obtained using a Norelco constant potential diffraction unit, type number 12045, equipped with a wide range goniometer type No. 42202, chromium tube type No. 32116, Geiger counter type No. 34473; all coupled to the Norelco circuit panel type No. 12049. The chromium K alpha radiation was supplied by operating the tube at a constant potential of 40 kilovolts and a current of 10 milliamperes. A vanadium filter was used to remove K beta radiation. The Geiger tube detector was operated at 1575 volts. A 1° divergence, 0.006 inch receiving, and 1° scatter slits were used. Strip chart recordings used for identification were made with a scanning speed of 1° 2 theta per minute with a chart speed of one-half inch per minute. A time constant of 2 seconds and a full scale chart reading of 100 counts per second was used. Under the above conditions, the patterns noted below were found.

The values of  $I/I_1$  noted are those for  $\text{NiFe}_2\text{O}_4$ . A small amount of  $\alpha\text{Fe}_2\text{O}_3$  was found in the patterns. The data is reported in the table.

Table

|    | $d$ : | $I/I_1$ |
|----|-------|---------|
| 5  | 4.82  | 14      |
|    | 2.948 | 31      |
|    | 2.698 | weak    |
| 10 | 2.513 | 100     |
|    | 2.406 | 13      |
|    | 2.082 | 23      |
|    | 1.702 | 10      |
| 15 | 1.606 | 24      |
|    | 1.474 | 40      |
|    | 1.453 | weak    |
|    | 1.318 | 4       |

#### EXAMPLE 2

20 The general procedure of Example 1 was repeated with the exception that potassium chloride was not used in the formation of the nickel ferrite. The yield of butadiene-1,3 was 63 mol percent.

#### EXAMPLE 3

25 A nickel ferrite catalyst was prepared from nickel carbonate and hydrated yellow ferric iron oxide. The ratio of ingredients was such that there were two atoms of iron per atom of nickel. The nickel carbonate and iron oxide 30 were thoroughly mixed in an aqueous slurry and the slurry thereafter was dried. The dry cake was broken into lumps and a 4 to 8 mesh fraction was reacted for 30 minutes at 950° C. to form the nickel ferrite. The catalyst was evaluated for the dehydrogenation of butene-2 35 to butadiene-1,3. A stainless steel reactor one inch in diameter was used and 20 cc. of the 4 to 8 mesh catalyst was utilized. 30 mols of steam and 0.6 mol of  $O_2$  (fed as air) were fed per mol of butene-2. The flow rate of butene-2 was 1.0 LHSV. At a reactor temperature of 40 400° C., the selectivity to butadiene was greater than 90 mol percent of the butene consumed.

#### EXAMPLE 4

45 Example 3 was repeated with the exception that the catalyst contained 2.5 atoms of iron per atom of nickel. At a reactor temperature of 400° C., the conversion was 64 percent and the selectivity to butadiene was 93 percent.

#### EXAMPLE 5

50 Example 3 was repeated with the exception that the catalyst contained 1.67 atoms of iron per atom of nickel and the amount of oxygen used was increased to 0.75 mol of  $O_2$  per mol of butene-2 fed. At a reactor temperature of 400° C., the selectivity to butadiene-1,3 was 86 percent.

#### EXAMPLE 6

55 The procedure of Example 1 was repeated using the catalyst of Example 1. Additionally, 0.03 mol of bromine (fed as an aqueous solution of HBr) per mol of butene-60 was fed to the reactor. Oxygen was fed at a rate of 0.85 mol of  $O_2$  per mol of butene and steam was employed in a ratio of 20 mols of steam per mol of butene fed. The flow rate of butene was 0.6 LHSV. At a reactor temperature of 550° C., the yield of butadiene was 74 mol percent per pass.

65 When an equivalent amount of iodine and chlorine were substituted for the bromine in Example 6, excellent yields of butadiene-1,3 were obtained.

70 The catalysts are not limited to those illustrated in the examples. Other methods of preparation and other compositions may be employed. The atoms of iron will preferably be present in an amount from about 20 to 95 weight percent, based on the total weight of the atoms of iron and nickel in the catalyst surface, but generally will be between 75 40 and 90 and a preferred ratio is from 50 to 85 weight

<sup>1</sup> Vycor is the trade name of Corning Glass Works, Corning, N.Y., and is composed of approximately 96 percent silica with the remaining being essentially  $\text{B}_2\text{O}_3$ .

percent iron. Particularly preferred are catalysts having a weight percent of iron from or about 55 to 81 percent by weight iron based on the total weight of atoms of iron and nickel. Valuable catalysts were produced comprising as the main active constituents iron, nickel and oxygen in the catalytic surface exposed to the reaction gases. High yields of product are obtained with catalysts having iron as the predominant metal in the catalytic surface. Preferably at least about 50 and generally at least about 65 weight percent of the atoms of nickel and iron will be present as nickel ferrite. Included in the definition of ferrites are the active intermediate oxides. The preferred nickel ferrite has a cubic face-centered crystal structure. Ordinarily the nickel ferrite will not be present in the most highly oriented crystalline structure, because it has been found that superior results may be obtained with catalysts wherein the nickel ferrite is relatively disordered, that is where there are defects in the crystalline structure. The desired catalyst may be obtained by conducting the reaction to form the active catalyst at relatively low temperatures, that is, at temperatures lower than some of the very high temperatures used for the formation of nickel ferrite prepared for semi-conductor applications. Generally the temperature of reaction for the formation of the catalyst comprising nickel ferrite will be less than 1300° C. and preferably less than 1150° C. Of course, under certain conditions momentary temperatures above these temperatures might also be permissible. The reaction time at the elevated temperature in the formation of the catalyst may preferably be from about five minutes to four hours at elevated temperatures high enough to cause formation of nickel ferrite but less than about 1150° C. Any iron not present in the form of nickel ferrite will desirably be present predominantly as gamma iron oxide. The alpha iron oxide will preferably be present in an amount of no greater than 40 weight percent of the catalytic surface, such as no greater than about 30 weight percent.

Although excellent results are obtained with the catalysts of this invention with a feed containing only the hydrocarbon, oxygen and perhaps steam or a diluent, it is one of the advantages of this invention that halogen may also be added to the reaction gases to give excellent results. The addition of halogen to the feed is particularly effective when the hydrocarbon to be dehydrogenated is saturated.

The source of halogen fed to the dehydrogenation zone may be either elemental halogen or any compound of halogen which would liberate halogen under the conditions of reaction. Suitable sources of halogen are such as hydrogen iodide, hydrogen bromide and hydrogen chloride; aliphatic halides such as ethyl iodide, methyl bromide, 1,2-dibromo ethane, ethyl bromide, amyl bromide and allyl bromide; cycloaliphatic halides such as cyclohexylbromide; aromatic halides such as benzyl bromide; halohydrins such as ethylene bromohydrin; halogen substituted aliphatic acids such as bromoacetic acid; ammonium iodide; ammonium bromide; ammonium chloride; organic amine halide salts such as methyl amine hydrobromide; and the like. Mixtures of various sources of halogen may be used. The preferred sources of halogen are iodine, bromine and chlorine and compounds thereof such as hydrogen bromide, hydrogen iodide, hydrogen chloride, ammonium bromide, ammonium iodide, ammonium chloride, alkyl halides of one to six carbon atoms and mixtures thereof, with the iodine and bromine compounds being particularly preferred, and the best results having been obtained with ammonium iodide, bromide or chloride. When terms such as halogen liberating materials or halogen materials are used in the specification and claims, this includes any source of halogen such as elemental halogens, hydrogen halides or ammonium halides. The amount of halogen, calculated as elemental halogen, may be as little as about 0.0001 or less mol of halogen per mol of the hydrocarbon compound to be dehydrogenated to as high as 0.2 or 0.5

or higher. The preferred range is from about 0.001 to 0.09 mol of halogen per mol of the hydrocarbon to be dehydrogenated.

Improved catalysts may be obtained by reducing the catalyst of the invention. The reduction of the catalyst may be accomplished prior to the initial dehydrogenation, or the catalyst may be reduced after the catalyst has been used. It has been found that a used catalyst may be regenerated by reduction and, thus, even longer catalyst life obtained. The reduction may be accomplished with any gas which is capable of reducing iron oxide to a lower valence such as hydrogen, carbon monoxide or hydrocarbons. Generally the flow of oxygen will be stopped during the reduction step. The temperature of reduction may be varied but the process is most economical at temperatures of at least about 200° C., with the upper limit being about 750° C. or 900° C. or even higher under certain conditions.

The preferred catalyst surface will generally have X-ray diffraction peaks at *d* spacings within or about 4.79 to 4.85, 2.92 to 2.98, 2.48 to 2.54, 2.05 to 2.11, 1.57 to 1.63, and 1.44 to 1.49, with the most intense peak being between 2.48 to 2.54. Particularly preferred catalysts will have *d* spacings within or about 4.80 to 4.84, 2.93 to 2.97, 2.50 to 2.53, 2.07 to 2.10, 1.59 to 1.61, and 1.46 to 1.49, with the most intense peak falling within or about 2.50 to 2.53. These X-ray determinations are suitably run with a cobalt tube.

We claim:

- 30 1. A process for the dehydrogenation of hydrocarbons having at least four carbon atoms which comprises contacting in the vapor phase at a temperature of greater than 250° C. a mixture of the said hydrocarbon to be dehydrogenated and from 0.2 to 2.5 mols of oxygen per mol of the said hydrocarbon with a catalyst for the dehydrogenation comprising nickel and iron wherein the atoms of iron are present in an amount of about 20 to 90 weight percent based on the total weight of the atoms of iron and nickel, to produce a dehydrogenated hydrocarbon product having the same number of carbon atoms as the said hydrocarbon.
- 35 2. A process for the dehydrogenation of hydrocarbons having at least four carbon atoms which comprises contacting in the vapor phase at a temperature of greater than 250° C. a mixture of the said hydrocarbon to be dehydrogenated and from 0.2 to 2.5 mols of oxygen per mol of the said hydrocarbon with a catalyst for the dehydrogenation comprising nickel ferrite to produce a dehydrogenated hydrocarbon product having the same number of carbon atoms as the said hydrocarbon.
- 40 3. A process for the dehydrogenation of hydrocarbons having from 4 to 5 carbon atoms which comprises contacting in the vapor phase at a temperature of greater than 250° C. a mixture of the said hydrocarbon to be dehydrogenated and from 0.2 to 2.5 mols of oxygen per mol of the said hydrocarbon with a catalyst for the dehydrogenation comprising nickel ferrite wherein the atoms of iron are present in an amount of about 40 to 90 weight percent based on the total weight of the atoms of iron and nickel, to produce a dehydrogenated hydrocarbon product having the same number of carbon atoms as the said hydrocarbon, the initial partial pressure of the said hydrocarbon being equivalent to less than one-half atmosphere at a total pressure of one atmosphere.
- 45 4. A process for the dehydrogenation of a hydrocarbon selected from the group consisting of n-butene, n-butane and mixtures thereof which comprises contacting in the vapor phase at a temperature of greater than about 325° C. a mixture of the said hydrocarbon to be dehydrogenated and from about 0.25 to about 1.6 mols of oxygen per mol of the said hydrocarbon with a catalyst for the dehydrogenation comprising nickel ferrite to produce a dehydrogenated hydrocarbon product having the same number of carbon atoms as the said hydrocarbon, the initial partial pressure of the said hydrocarbon being
- 50
- 55
- 60
- 65
- 70

equivalent to less than one-half atmosphere at a total pressure of one atmosphere.

5. A process for the dehydrogenation of aliphatic hydrocarbons having at least four carbon atoms which comprises contacting in the vapor phase at a temperature of from about 325° C. to 525° C. a mixture of the said hydrocarbon to be dehydrogenated and from 0.2 to 1.6 mols of oxygen per mol of the said hydrocarbon with a catalyst for the dehydrogenation comprising nickel and iron wherein the atoms of iron are present in an amount of 50 to 85 weight percent based on the total weight of the atoms of iron and nickel, to produce a dehydrogenated hydrocarbon product having the same number of carbon atoms as the said hydrocarbon, the initial partial pressure of the said hydrocarbon being equivalent to less than one-half atmosphere at a total pressure of one atmosphere.

6. A process for the dehydrogenation of aliphatic hydrocarbons having at least four carbon atoms which comprises contacting in the vapor phase at a temperature of greater than 325° C. a mixture of the said hydrocarbon to be dehydrogenated from 0.2 to 2.5 mols of oxygen per mol of the said hydrocarbon and from 2 to 40 mols of steam per mol of the said hydrocarbon with a catalyst for the dehydrogenation comprising nickel ferrite to produce a dehydrogenated hydrocarbon product having the same number of carbon atoms as the said hydrocarbon.

7. A process for the dehydrogenation of aliphatic hydrocarbons having at least four carbon atoms which comprises contacting in the vapor phase at a temperature of greater than 325° C. a mixture of the said hydrocarbon to be dehydrogenated and from 0.2 to 2.5 mols of oxygen per mol of the said hydrocarbon with an autoregenerative catalyst for the dehydrogenation comprising nickel and iron wherein the atoms of iron are present in an amount of 55 to 81 weight percent based on the total weight of the atoms of iron and nickel, to produce a dehydrogenated hydrocarbon product having the same number of carbon atoms as the said hydrocarbon, the initial partial pressure of the said hydrocarbon being equivalent to less than one-half atmosphere at a total pressure of one atmosphere.

8. A process for the dehydrogenation of hydrocarbons having from 4 to 5 carbon atoms which comprises contacting in the vapor phase at a temperature of at least about 375° C. a mixture of the said hydrocarbon to be dehydrogenated and from 0.35 to 1.2 mols of oxygen per mol of the said hydrocarbon with a catalyst for the dehydrogenation comprising nickel ferrite wherein the atoms of iron are present in an amount of 55 to 81 weight percent based on the total weight of the atoms of iron and nickel, to produce a dehydrogenated hydrocarbon product having the same number of carbon atoms as the said hydrocarbon, the initial partial pressure of the said hydrocarbon being equivalent to less than one-third atmosphere at a total pressure of one atmosphere.

9. A process for the dehydrogenation of a hydrocarbon selected from the group consisting of n-butene, n-butane and mixtures thereof which comprises contacting in the vapor phase at a temperature of from 375° C. to 525° C. and at a pressure of 4 p.s.i.a. to 125 p.s.i.a. a mixture of the said hydrocarbon to be dehydrogenated and from about 0.25 to about 1.6 mols of oxygen per mol of the said hydrocarbon with a catalyst for the dehydrogenation comprising nickel ferrite to produce a dehydrogenated hydrocarbon product having the same number of carbon atoms as the said hydrocarbon, the initial partial pressure of the said hydrocarbon being equivalent to less than one-fifth atmosphere at a total pressure of one atmosphere.

10. A process for the dehydrogenation of butene to butadiene-1,3 which comprises contacting in the vapor phase at a temperature of from 375° C. to 575° C. and at a total pressure of less than 75 p.s.i.a. a mixture of the said butene, from 8 to about 35 mols of steam and from 0.35 to 1.2 mols of oxygen per mol of the said

butene with a catalyst for the dehydrogenation comprising nickel ferrite wherein the atoms of iron are present in an amount of 55 to 81 weight percent based on the total weight of the atoms of iron and nickel, to produce butadiene-1,3.

11. A process for the vapor phase dehydrogenation of aliphatic hydrocarbons having at least four carbon atoms which comprises contacting in the vapor phase at a temperature of greater than 250° C. a mixture of the said hydrocarbon to be dehydrogenated, from 0.2 to 2.5 mols of oxygen per mol of the said hydrocarbon and a halogen with a catalyst for the dehydrogenation comprising nickel ferrite wherein the atoms of iron are present in an amount of about 40 to 90 weight percent based on the total weight of the atoms of iron and nickel, to produce a dehydrogenated hydrocarbon product having the same number of carbon atoms as the said hydrocarbon, the initial partial pressure of the said hydrocarbon being equivalent to less than one-half atmosphere at a total pressure of one atmosphere.

12. A process for the dehydrogenation of aliphatic hydrocarbons having from 4 to 5 carbon atoms which comprises contacting in the vapor phase at a temperature of greater than 325° C. a mixture of the said hydrocarbon to be dehydrogenated, from 0.25 to 1.6 mols of oxygen per mol of the said hydrocarbon and from 0.0001 to 0.2 mols of halogen per mol of the said hydrocarbon with an autoregenerative catalyst for the dehydrogenation comprising nickel ferrite wherein the atoms of iron are present in an amount of about 40 to 90 weight percent based on the total weight of the atoms of iron and nickel, to produce a dehydrogenated hydrocarbon product having the same number of carbon atoms as the said hydrocarbon, the initial partial pressure of the said hydrocarbon being equivalent to less than one-half atmosphere at a total pressure of one atmosphere.

13. A process for the dehydrogenation of aliphatic hydrocarbons having from 4 to 5 carbon atoms which comprises contacting in the vapor phase at a temperature of greater than 325° C. a mixture of the said hydrocarbon to be dehydrogenated, from 0.25 to 1.6 mols of oxygen per mol of the said hydrocarbon with an autoregenerative catalyst for the dehydrogenation comprising nickel ferrite wherein the atoms of iron are present in an amount of about 40 to 90 weight percent based on the total weight of the atoms of iron and nickel, to produce a dehydrogenated hydrocarbon product having the same number of carbon atoms as the said hydrocarbon, the initial partial pressure of the said hydrocarbon being equivalent to less than one-half atmosphere at a total pressure of one atmosphere.

14. A process for the dehydrogenation of butene to butadiene-1,3 which comprises feeding to a reactor in the vapor phase at a temperature of at least 250° C. a gaseous mixture of the said butene and from 0.35 to 1.2 mols of oxygen per mol of the said butene with an autoregenerative catalyst for the dehydrogenation comprising nickel and iron wherein the atoms of iron are present in an amount of about 2 atoms of iron per atom of nickel based on the total weight of the atoms of iron and nickel, to produce butadiene-1,3, the initial partial pressure of the said butene being equivalent to less than one-fifth atmosphere at a total pressure of one atmosphere.

15. A process for the dehydrogenation of aliphatic hydrocarbons having at least four carbon atoms which comprises contacting in the vapor phase at a temperature of greater than 250° C. a mixture of the said hydrocarbon to be dehydrogenated and from 0.2 to 2.5 mols of oxygen per mol of the said hydrocarbon with a catalyst for the dehydrogenation comprising nickel ferrite to produce a dehydrogenated hydrocarbon product having the same number of carbon atoms as the said hydrocarbon, the initial partial pressure of the said hydrocarbon being equivalent to less than one-half atmosphere at a total

pressure of one atmosphere, said catalyst having been reduced with a reducing gas.

16. A process for the preparation of butadiene-1,3 which comprises contacting in the vapor phase at a temperature of 375° C. to 525° C. and at a total pressure of about 4 p.s.i.a. to 100 p.s.i.a. a mixture of n-butene and from 0.35 to 1.2 mols of oxygen and from 8 to 35 mols of steam per mol of the said n-butene with an auto-regenerative catalyst for the dehydrogenation comprising nickel ferrite wherein the atoms of iron are present in amount of 55 to 81 weight percent based on the total weight of the atoms of iron and nickel with any iron not present in the form of nickel ferrite being predominantly present as gamma iron oxide to produce butadiene-1,3.

17. A process for the preparation of butadiene-1,3 which comprises contacting in the vapor phase at a temperature of 375° C. to 525° C. and at a total pressure of about 4 p.s.i.a. to 100 p.s.i.a. a mixture of n-butene and from 0.35 to 1.2 mols of oxygen and from 8 to 35

5 mols of steam per mol of the said n-butene with an auto-regenerative catalyst for the dehydrogenation comprising nickel ferrite wherein the atoms of iron are present in an amount of 55 to 81 weight percent based on the total weight of the atoms of iron and nickel with any iron not present in the form of nickel ferrite being predominantly present as gamma iron oxide to produce butadiene-1,3, and after the yield of butadiene-1,3 has fallen off after continued use regenerating the catalyst by reducing 10 the catalyst with hydrogen.

References Cited by the Examiner

UNITED STATES PATENTS

|    |           |        |                       |           |
|----|-----------|--------|-----------------------|-----------|
| 15 | 3,168,587 | 2/1965 | Michaels et al. ----- | 260—683.3 |
|    | 3,179,707 | 4/1965 | Lee -----             | 260—669   |
|    | 3,207,811 | 9/1965 | Bajars -----          | 260—680   |

DELBERT E. GANTZ, Primary Examiner.

20 G. E. SCHMITKONS, Assistant Examiner.